

[54] PROCESS OF FORMING SILVER TRANSFER IMAGES

[75] Inventors: Robrecht Julius Thiers, Brasschaat; Josef Frans Willems, Urbijk; Roger Alois Spriet, Edegem, all of Belgium

[73] Assignee: Gevaert-Agfa N.V., Mortsel, Germany

[22] Filed: Oct. 12, 1970

[21] Appl. No.: 80,151

[30] Foreign Application Priority Data

Oct. 27, 1969 Great Britain.....52,571/69

[52] U.S. Cl. ....96/29 R

[51] Int. Cl. ....G03c 5/54

[58] Field of Search.....96/29, 76

[56]

References Cited

UNITED STATES PATENTS

3,189,454 6/1965 Luckey et al.....96/95  
3,458,316 7/1969 Viro .....96/94

Primary Examiner—J. Travis Brown

Assistant Examiner—John L. Goodrow

Attorney—Brufsky, Staas, Breiner and Halsey

[57]

ABSTRACT

A process for the production of silver images according to the silver complex diffusion transfer process carried out in the presence of a hydroxylamine derivative developing agent and a (poly)amino(poly)carboxylic acid sequestering agent in acid form or in the form of a water-soluble salt is described. Better quality transfer images at substantially lower illumination levels are realized.

12 Claims, No Drawings

## PROCESS OF FORMING SILVER TRANSFER IMAGES

The present invention relates to the formation of silver images by the silver complex diffusion transfer process.

Processes for forming silver images by the steps of image-wise exposure and development of a photosensitive silver halide element, the formation of a diffusible complex of unexposed silver halide in the unexposed areas of the said photosensitive element and the transfer by diffusion of said complex to an element, in superposed relationship with the photosensitive element, where the silver of said complex is precipitated or reduced to form a visible image, are now well known.

The element to which the silver complex is transferred is often referred to as the image-receiving element and generally comprises agents, known as development nuclei, that promote the precipitation of the silver of said silver complex.

According to a typical embodiment of the silver complex diffusion transfer process suitable for in-camera processing a composite material of unitary structure is used which comprises a photosensitive element, an image-receiving element and a viscous processing fluid contained in a pod or container. After image-wise exposure of the photosensitive element, which comprises a silver halide emulsion layer, the superposed elements i.e., the photosensitive element and the image-receiving element are guided between a pair of pressure rollers whereby the viscous processing liquid is spread as a uniform layer between the photosensitive element and the image-receiving element.

The photosensitive element and the image-receiving element are maintained in superposed relation for a determined period, usually of the order of 10 to 120 seconds, during which the exposed silver halide is developed, the undeveloped silver halide is converted into a water-soluble complex silver salt and the said complex is transferred through the layer of processing liquid to the silver precipitating layer of the image-receiving element where it is converted into a visible print. At the end of this contact period the photosensitive element is separated by stripping from the image-receiving element. Elements suitable for use in this silver complex diffusion transfer process are described in detail e.g., in U.S. Pat. No. 2,543,181 of Edwin H. Land, issued Feb. 27, 1951.

A wide variety of silver halide developing agents and silver halide complexing agents, are known for use in such diffusion transfer processes.

As silver halide developing agents it has been proposed amongst others in U.S. Pat. No. 2,857,276 of Edwin H. Land and Helen J. Tracy, issued Oct. 21, 1958 to use hydroxylamine and derivatives thereof, of which the oxidation products leave no residual stain in the positive silver image obtained. Hydroxylamine itself is less suitable because it gives rise to fog but the N,N-dialkylhydroxylamines such as N,N-diethylhydroxylamine and the heterocyclic N-hydroxylamines such as N-hydroxymorpholine, N-hydroxypiperidine and N-hydroxypyrrolidine disclosed in the above U.S. Pat specification are particularly suitable. Other hydroxylamine derivatives that have been proposed for use as silver halide developing agents and of which the

development activity is higher than that of the N,N-dialkylhydroxylamines include for example aminoalkylhydroxylamines, more especially N,N-dialkylhydroxylamines having in at least one of the N-alkyl groups an intralinear amino nitrogen atom, either cyclic or acyclic, examples of which can be found in U.S. Pat. No. 3,287,125, of Milton Green, Adnan A. Sayigh and Henri Ulrich, issued Nov. 22, 1966, alkoxy hydroxylamines, more especially N,N-dialkyl hydroxylamines of which at least one of the N-alkyl groups is substituted by alkoxy or alkoxy-alkoxy, examples of which can be found in U.S. Pat. No. 3,293,034 of Milton Green, Adnan A. Sayigh and Henri Ulrich, issued Dec. 20, 1966 and sulphone hydroxylamines, more especially N,N-dialkyl hydroxylamines having in at least one of the N-alkyl groups an intralinear sulphonyl (—SO<sub>2</sub>—) group, examples of which can be found in U.S. Pat. No. 3,287,124 of Milton Green, Adnan A. Sayigh and Henri Ulrich, issued Nov. 22, 1966.

It has now been found when using, in a process for the production of silver images according to the silver complex diffusion transfer process, carried out developing agent, a photosensor element the presence of a hydroxylamine derivative as silver halide emulsion comprising a silver halide emulsion layer, and a (poly)amino(poly)carboxylic acid sequestering compound, in acid form or in the form of a water-soluble salt, transfer images are obtained of improved quality.

The use of (poly)amino(poly)carboxylic acid sequestering compounds, in acid form or in the form of a water-soluble salt, in a silver complex diffusion transfer process wherein use is made of a hydroxylamine developing agent is effective to give better quality transfer images at substantially lower illumination levels than are necessary in the absence of said compounds, without giving rise to a noteworthy decrease in maximum density of the images formed.

Therefore, in accordance with the present invention, there is provided a process of forming silver transfer images which comprises the steps of exposing a photosensitive element containing a silver halide emulsion layer and a (poly)amino(poly) carboxylic acid sequestering compound, in acid form or in the form of a water-soluble salt, developing the exposed photosensitive silver halide emulsion layer and forming a soluble silver complex of unexposed silver halide by treating the said photosensitive silver halide emulsion layer with an alkaline processing fluid in the presence of a hydroxylamine developing agent and a silver halide complexing agent, transferring said soluble silver complex by diffusion to the silver receptive layer of an image-receiving element in superposed relationship with said silver halide emulsion, forming at said silver receptive layer an image incorporating silver from said silver complex, and separating said image-receiving element from said photosensitive element.

Examples of suitable (poly)amino(poly)carboxylic acid sequestering compounds as well as details about the preparation of said sequestering compounds can be found in Ind. Chim. Belg. Tome XXI (1956) p. 338-346 and in Ind. Chim. Belg. Tome XXIII (1958) p. 1,105-1,115.

Particularly suitable (poly)amino(poly)carboxylic acids for use in acid or salt form in accordance with the present invention can be represented by the following non-limitative general formula:



wherein:

L stands for alkylene including substituted alkylene e.g., hydroxyalkylene, cycloalkylene including substituted cycloalkylene or alkylene interrupted by one or more hetero atoms, such as an oxygen atom,

x represents 0, 1 or 2,

R stands for lower alkylene e.g., methylene and ethylene including substituted lower alkylene e.g., alkylene substituted by alkyl, aryl, aralkyl, including substituted alkyl, aryl and aralkyl, and

each of R<sub>1</sub> and R<sub>2</sub> (the same or different) stands for hydrogen, lower alkyl including substituted lower alkyl, aralkyl including substituted aralkyl or aryl including substituted aryl; examples of substituted alkyl groups for R<sub>1</sub> and for R<sub>2</sub> are alkyl substituted with hydroxyl, halogen, alkoxy, carbamoyl, amino, substituted amino e.g., dihydroxyalkylamino, epoxy, carboxyl, sulpho, phosphono, mercapto, alkylmercapto, alkoxy carbonyl, a nitrogen-containing heterocyclic ring e.g., pyridyl and examples of substituted aryl groups and aralkyl groups for R<sub>1</sub> and/or R<sub>2</sub> are: aryl and aralkyl substituted by hydroxyl, halogen, alkyl, alkoxy, nitro, carboxyl and sulpho.

The following is a non-limitative list of examples of (poly)amino(poly)carboxylic acids corresponding to the above general formula:



ethylenediamine, N,N,N',N'-tetraacetic acid disodium salt



1,2-propylenediamine, N,N,N',N'-tetraacetic acid



ethylenediamine, N,N,N',N'-tetrapropionic acid



N-(2-hydroxyethyl)-ethylenediamine, N,N',N'-triacetic acid



N-(2-hydroxypropyl)-ethylenediamine, N,N'-triacetic acid



N-(2,3-dihydroxypropyl)-ethylenediamine, N,N',N'-triacetic acid



N,N'-di(2-hydroxyethyl)-ethylenediamine, N,N'-diacetic acid



diethylenetriamine, N,N,N',N'',N'''-pentaacetic acid



nitrilo triacetic acid



ethylenediamine, N,N'-di(o-hydroxyphenyl)acetic acid



di(2-hydroxyethyl)-amino acetic acid



2-hydroxyethyl-amino diacetic acid



1,2-amino cyclohexane, N,N,N',N'-tetraacetic acid



2,3-dihydroxypropyl-aminodiacetic acid



ethyleneglycol bis(2-aminoethyl)-N,N,N',N'-tetraacetic acid



N-(2-hydroxyethyl)-N'-(alpha-pyridinomethyl)-ethylenediamine, N,N'-diacetic acid



In a process for preparing silver transfer images according to the present invention wherein compounds corresponding to the above general formula are used, the said compounds are present in the photosensitive element. These compounds may be located in the silver halide emulsion layer of said element or in a layer in water-permeable relationship with said emulsion layer. They may be used in amounts varying between very wide limits, preferably, they are used in amounts comprised between 30 mg and 15 g per mole of silver halide.

The silver halide emulsions utilized in preparing photosensitive elements used in the present diffusion transfer system can be any of the conventional negative-type emulsions. Typical suitable silver halides include silver chloride, silver bromide, silver

bromide, silver chloroiodide, silver chlorobromide, silver chlorobromochloride, etc. These silver halide emulsions can contain spectral sensitizers, speed-increasing addenda, hardeners, coating aids, antifogants, plasticizers and the like conventional emulsion addenda.

The photosensitive silver halide element may also comprise in the silver halide emulsion layer or in a layer in water-permeable relationship with the said emulsion layer, compounds having a favorable effect on the maximum density of the image formed and/or in the speed of the photosensitive element. Examples of these compounds are the 1-aryl-3-pyrazolidinone compounds examples of which can be found in the application for "Silver Complex Diffusion Transfer Process" filed on even date herewith (=United Kingdom Patent application No. 52,572/69), as well as diamine or polyamine compounds and morpholine derivatives, typical examples of which are the compounds represented by the following formulas:

- a.  $\text{H}_2\text{N}-\text{CH}_2-\text{CH}_2-\text{CH}_2-\text{NH}-\text{CH}_2-\text{CH}_2-\text{NH}_2$   
25 b.  $\text{H}_2\text{N}-(\text{CH}_2)_2-\text{NH}-(\text{CH}_2)_2-\text{NH}-(\text{CH}_2)_2-\text{NH}_2$   
c.  $\text{H}_2\text{N}-(\text{CH}_2)_2-\text{NH}-(\text{CH}_2)_2-\text{NH}_2$   
d.  $\text{H}_2\text{N}-\text{CH}_2-\text{CH}_2-\text{NH}-\text{CH}_2-\text{CH}_2-\text{OH}$





As previously noted, processing occurs with an alkaline processing liquid in the presence of a silver halide complexing agent and a hydroxylamine developing



20 agent. These agents are preferably present in the processing liquid itself although it is also possible to incorporate them in the photosensitive or image-receiving element. For instance, the hydroxylamine derivatives can be incorporated in the said elements in the 25 form of acid salts thereof e.g., in hydrochloride or hydrobromide form. When the developing and/or silver complexing agents are incorporated in the photosensitive and/or image-receiving element, the development of the exposed silver halide and the formation of the 30 silver complex of unexposed silver halide is activated when the alkaline processing fluid is spread as a thin layer between the photosensitive element and the image-receiving element.

Silver halide complexing agents suitable for use in 35 diffusion transfer processes are well known in the art and include alkali metal thiosulphates and thiocyanates, such as sodium thiosulphate and sodium thiocyanate. Silver halide complexing agents that are particularly suitable for use in accordance with the present 40 invention are cyclic imides for example barbituric acid, uracil and urazole as well as derivatives thereof, examples of which can be found in U.S. Pat. No. 2,857,276 mentioned above. Among the hydroxylamine developing agents that are particularly suitable, mention may 45 be made of the heterocyclic N-hydroxylamines such as N-hydroxymorpholine, N-hydroxy piperidine and N-hydroxy pyrrolidine, the primary and secondary N-lower alkyl hydroxylamines such as N,N-diethylhydroxylamine, the alkoxy-substituted derivatives thereof such as N,N-di(2-ethoxyethyl) hydroxylamine and N-ethyl-N-(2-ethoxyethyl)-hydroxylamine, the sulphone-hydroxylamines such as N-methyl-N-2-ethylsulphonyl-ethyl hydroxylamine and bis-2-(methyl-hydroxylamino)-ethyl sulphone and the aminoalkyl hydroxylamines such as N-methyl-N-2-dimethylaminoethyl-hydroxylamine. Further examples of such hydroxylamine derivatives can be found in the U.S. patent specifications referred to above.

60 The processing fluid comprises bases imparting to the fluid the required alkalinity. As examples of such bases mention may be made of alkali-metal hydroxides, e.g., sodium and potassium hydroxide, sodium carbonate, borax, sodium metaborate, trisodium phosphate, etc.

The fluid may further contain, or dissolve in its travel to the photosensitive element, other compounds which

are desired in the treatment of the photosensitive layer and in the production of the positive image in the image-receiving layer.

In silver complex diffusion transfer processes for in-camera processing, the processing fluid employed is relatively viscous, of the order of 1,000 to 200,000 centipoises at 20°C, so as to be easily controlled when spread. In order to obtain the desired viscosity, the liquid contains a thickening agent, preferably a water-soluble film-forming material such as water-soluble plastic so that when the liquid is removed from the processing layer by absorption and/or evaporation there remains a solid plastic film. The film-forming plastic may be any of the high molecular weight polymers which are stable to alkali and which are soluble in aqueous alkaline solutions e.g., hydroxyethylcellulose, starch or gum, polyvinylalcohol, the sodium salts of polymethacrylic acid and polyacrylic acid, sodium alginate, sodium carboxymethyl cellulose. As is known in the art, stripping of the silver halide element from the image-receiving element may separate the solidified layer of processing composition from the image-receiving element or may permit the layer of processing composition to remain in contact with the image-receiving element so that the solidified layer provides a protective coating over the image obtained.

The viscous processing fluid for use in in-camera processing is preferably confined within a hermetically sealed container or pod which is positioned between the photosensitive element and the image-receiving element and which is ruptured and releases its contents upon advancing the photosensitive element and image-receptive element between a pair of pressure-rollers. Such a container is impervious to the processing liquid and to the vapor of said liquid, and may be formed of a multilayer composite material comprising as inner layer in contact with the liquid, a material which is impervious to the liquid as intermediate layer a substance which is impervious to the vapor of said liquid and as outer layer a material merely serving as a backing or support. In its preferred form, the container is formed of a multilayer material whose inner layer is formed of a plastic such as polyvinyl acetal e.g., polyvinyl butyral, polymeric esters such as cellulose acetate, cellulose acetate butyrate, polyvinyl acetate, polyvinyl chloride, etc., said layer being backed by a metal foil e.g., a lead foil or lead-tin foil which is impervious to the vapors of said solution. The containers may be strengthened by a more rapid backing material such as kraft paper or a plastic such as polyvinyl acetate and polyvinyl chloride. More details as to the construction of such a rupturable container can be found amongst others in U.S. Pat. No. 2,634,886 of Edwin H. Land, issued Apr. 14, 1953.

The silver halide emulsion layer and/or the image-receiving layer may be coated on opaque or transparent supports. In this way it is possible to expose the photosensitive element from either side as desired and it is possible to form either reflection prints or transparencies.

The image-receiving layer of the image-receiving element preferably comprises mentioned, promoting precipitation of the silver from the transferred silver complex. Examples of such agents, called development nuclei or shortly nuclei, are well known and include sulphides, selenides, polysulphides, polyselenides, thioureas, thioacetamides, mercaptans, stannous halides, heavy metals or their salts and fogged silver halide. Sulphides of heavy metals such as of antimony,

bismuth, cadmium, cobalt, lead, nickel and silver are also suited. Lead sulphide and zinc sulphide as well as the complex salts thereof are especially effective either in themselves or mixed with thioacetamide, dithiobiuret and dithio-oxamide. Among the heavy metals silver, gold, platinum, palladium and mercury are to be mentioned preferably in colloidal form.

The development nuclei may be associated with a granular, inorganic, water-soluble, substantially chemically inert substance such as silica as vehicle for the said nuclei whereby aggregation of the precipitated silver is promoted.

In at least one layer of the image-receiving element other substances may also be incorporated which play a part in the formation of the diffusion transfer image e.g., black-toning agents, anti-yellowing agents, optical bleaching agents, softening agents, etc.

For in-camera processing the image-receiving element may be constructed as described in U.S. Pat. No. 2,823,112 of Edwin H. Land, issued Feb. 11, 1958. According to this United States patent specification the print-receiving element is so constructed that the viscous processing fluid separates therefrom and leaves no droplets or film of developing composition on the print-receiving layer. The image-receiving layer is thin, holding a mass of water so small that there is not tactful wetness. Moreover, by making the print-receiving layer so thin the tendency to curl is also avoided. Consequently, when peeled from the photosensitive element, which carries the viscous processing layer, the image-receiving element appears to be a dry sheet.

According to this United States patent specification a layer, which is substantially impervious to the processing liquid and which may be the liquid-impervious surface of a supporting sheet which is entirely formed of liquid-impervious material is provided between the silver precipitating layer in which the positive is formed, and the remainder of the image-receiving element. Further, the image-receiving layer is provided with a surface from which the viscous film of processing fluid may be readily stripped. Thus, according to said United States patent specification the outer surface of the image-receiving element contacting the layer of processing composition is so constituted as to have a lesser adhesion for the solid residue of the liquid processing composition than does the photosensitive element. As a result, the photosensitive element, when stripped from the image-receiving element, carries with it the residue of the processing composition. Further, between the image-receiving layer and the stripping layer an abrasion resistant coating may be provided.

According to this United States patent specification stripping of the silver halide element from the image-receiving element separates the layer of processing solution from the image-receiving element. However, as noted hereinbefore in order to provide the image-receiving element with a protective coating, it is also possible that upon stripping the layer of processing solution remains in contact with the said image-receiving element. Such stripping techniques are taught in U.S. Pat. No. 2,647,056 of Edwin H. Land, issued July 28, 1953.

The following examples illustrate the present invention. In these examples the value given for the speed are relative values, measured at density 0.5.

#### EXAMPLE 1

A photosensitive element was prepared which com-

prises a silver bromoiodide emulsion layer applied to a paper support and containing per kg an amount of silver halide corresponding to 60 g of silver nitrate and a (poly)amino(poly)carboxylic acid compound as listed in the table below in the amount given. After exposure, the photosensitive element together with an image-receiving element comprising a silver receptive layer containing development nuclei dispersed in a matrix of colloidal silica coated on a water-impervious base according to the practice described in U.S. Pat. No. 2,823,122 of Edwin H. Land, issued Feb. 11, 1958, were advanced in superposed relationship between a pair of pressure applying rollers to spread between them in a thin layer a processing composition comprising per liter:

|                                     |       |
|-------------------------------------|-------|
| sodium carboxymethyl cellulose      | 40 g  |
| sodium hydroxide                    | 35 g  |
| uracil                              | 75 g  |
| N,N-di(2-ethoxyethyl)-hydroxylamine | 40 ml |

After a contact period of 36 seconds, the emulsion together with the layer of processing liquid was stripped from the image-receiving element to uncover the positive print.

The results obtained are listed in the table below.

TABLE

| Compound added per kg of emulsion | D <sub>max</sub> | D <sub>min</sub> | Gamma | Speed (%) |
|-----------------------------------|------------------|------------------|-------|-----------|
| none                              | 1.55             | 0.04             | 1.50  | 100       |
| 1 g of compound 1                 | 1.48             | 0.03             | 1.22  | 153       |
| 0.1 g of compound 1               | 1.52             | 0.03             | 1.37  | 130       |
| 0.1 g of compound 10              | 1.50             | 0.04             | 1.09  | 146       |
| 0.1 g of compound 12              | 1.52             | 0.03             | 1.32  | 142       |
| 0.1 g of compound 15              | 1.51             | 0.03             | 1.30  | 133       |
| 0.1 g of compound 25              | 1.53             | 0.03             | 1.44  | 124       |

These results show that the compounds of use according to the present invention have a favorable effect on the speed without causing a noteworthy decrease in maximum density of the image formed.

## EXAMPLE 2

Example 1 was repeated with the difference that the photosensitive elements were processed directly after preparation and after having been stored for 5 days at 45°C and 15 percent of relative humidity.

The following results were attained.

| Compound added per kg of emulsion | Fresh material   |                  |                       | Stored material  |                  |                       |
|-----------------------------------|------------------|------------------|-----------------------|------------------|------------------|-----------------------|
|                                   | D <sub>max</sub> | D <sub>min</sub> | Gamma Speed<br>ma (%) | D <sub>max</sub> | D <sub>min</sub> | Gamma Speed<br>ma (%) |
| none                              | 1.57             | 0.03             | 1.73 100              | 1.59             | 0.03             | 1.63 87               |
| 50 mg of compound 10              | 1.53             | 0.03             | 1.33 139              | 1.58             | 0.03             | 1.47 112              |
| 100 mg of compound 10             | 1.56             | 0.03             | 1.50 136              | 1.51             | 0.03             | 1.11 127              |
| 200 mg of compound 10             | 1.54             | 0.02             | 1.57 136              | 1.48             | 0.03             | 1.21 130              |
| 50 mg of compound 12              | 1.55             | 0.03             | 2.03 136              | 1.56             | 0.03             | 1.40 115              |
| 100 mg of compound 12             | 1.54             | 0.03             | 1.70 139              | 1.56             | 0.03             | 1.46 118              |
| 200 mg of                         |                  |                  |                       |                  |                  |                       |

|                       |      |      |      |     |      |      |      |     |
|-----------------------|------|------|------|-----|------|------|------|-----|
| compound 12           | 1.54 | 0.03 | 1.49 | 139 | 1.50 | 0.03 | 1.24 | 127 |
| 50 mg of compound 15  | 1.56 | 0.02 | 1.82 | 121 | 1.59 | 0.04 | 1.59 | 106 |
| 100 mg of compound 15 | 1.55 | 0.03 | 1.70 | 136 | 1.58 | 0.04 | 1.55 | 109 |
| 200 mg of compound 15 | 1.55 | 0.03 | 1.51 | 136 | 1.55 | 0.03 | 1.40 | 121 |

## EXAMPLE 3

Example 1 was repeated with the difference that the silver halide emulsion layer of the photosensitive element now comprises compound 24 in an amount of 1 g per kg of emulsion. The sensitometric results obtained, as compared with the results obtained when no compound 24 is present are the following:

| Material                        | D <sub>max</sub> | D <sub>min</sub> | Gamma | Speed(%) |
|---------------------------------|------------------|------------------|-------|----------|
| Comparison material             | 1.55             | 0.04             | 1.69  | 100      |
| Material comprising compound 24 | 1.53             | 0.04             | 1.32  | 138      |

## EXAMPLE 4

This example is analogous to example 3 with the only difference that the silver halide emulsion contains per kg in addition to 1 g of compound 24, 0.5 g of 1-phenyl-3-pyrazolidinone.

The following results were attained.

| Material                                                                  | Fresh material   |                  |                       | Material stored for 5 days at 49°C/15% R.H. |                  |                       |
|---------------------------------------------------------------------------|------------------|------------------|-----------------------|---------------------------------------------|------------------|-----------------------|
|                                                                           | D <sub>max</sub> | D <sub>min</sub> | Gamma Speed<br>ma (%) | D <sub>max</sub>                            | D <sub>min</sub> | Gamma Speed<br>ma (%) |
| Comparison material                                                       | 1.55             | 0.03             | 1.80 100              | 1.57                                        | 0.03             | 1.90 85               |
| Material comprising compound 24 and 0.5 g of 1-phenyl-3-pyrazolidinone    | 1.64             | 0.03             | 1.95 136              | 1.67                                        | 0.03             | 2.03 121              |
| Material comprising 0.5 g of 1-phenyl-3-pyrazolidinone and no compound 24 | 1.65             | 0.03             | 1.54 153              | 1.66                                        | 0.06             | 2.51 35               |

When comparing these results with the results obtained in example 3 it appears that 1-phenyl-3-pyrazolidinone has a favorable effect on the maximum density of the image formed and that the gain in speed by the presence of compound 24 is maintained though 1-phenyl-3-pyrazolidinone when used alone has a marked desensitizing effect after storage.

## EXAMPLE 5

This example is analogous to Example 1. The photosensitive element according to the invention now comprises in the silver halide emulsion layer 500 mg of compound 1 per kg of emulsion.

The following results were attained.

| Material              | Fresh material   |                  |                       | Material Stored for 5 days at 49°C/15% R.H. |                  |                       |
|-----------------------|------------------|------------------|-----------------------|---------------------------------------------|------------------|-----------------------|
|                       | D <sub>max</sub> | D <sub>min</sub> | Gamma Speed<br>ma (%) | D <sub>max</sub>                            | D <sub>min</sub> | Gamma Speed<br>ma (%) |
| none                  | 1.57             | 0.03             | 1.73 100              | 1.59                                        | 0.03             | 1.63 87               |
| 50 mg of compound 10  | 1.53             | 0.03             | 1.33 139              | 1.58                                        | 0.03             | 1.47 112              |
| 100 mg of compound 10 | 1.56             | 0.03             | 1.50 136              | 1.51                                        | 0.03             | 1.11 127              |
| 200 mg of compound 10 | 1.54             | 0.02             | 1.57 136              | 1.48                                        | 0.03             | 1.21 130              |
| 50 mg of compound 12  | 1.55             | 0.03             | 2.03 136              | 1.56                                        | 0.03             | 1.40 115              |
| 100 mg of compound 12 | 1.54             | 0.03             | 1.70 139              | 1.56                                        | 0.03             | 1.46 118              |
| 200 mg of             |                  |                  |                       |                                             |                  |                       |

|                                                     |      |      |      |     |      |      |      |     |
|-----------------------------------------------------|------|------|------|-----|------|------|------|-----|
| Comparison material comprising 500 mg of compound 1 | 1.58 | 0.05 | 1.49 | 100 | 1.62 | 0.04 | 1.95 | 73  |
|                                                     | 1.55 | 0.03 | 1.43 | 140 | 1.55 | 0.03 | 1.45 | 141 |

## EXAMPLE 6

By addition of 1-p-tolyl-4,4-dimethyl-5-ethoxy-3-pyrazolidinone, a compound as described and claimed in United Kingdom Patent application 52,572/69 referred to above, to the emulsion layer of the

5 approximately 10 percent).

## EXAMPLE 8

From Example 5 it appears that compound 1 has a favorable effect on the sensitivity without having a noteworthy influence on the maximum density of the image formed.

10 The results below show that when per kg of emulsion an amine is added in the amount given in the table below, in addition to 500 mg of compound 1, the speed can still be increased by approximately 25 percent.

| Compound added per kg. of emulsion                                                                                          | D <sub>max</sub> | D <sub>min</sub> | Gamma | Speed percent |
|-----------------------------------------------------------------------------------------------------------------------------|------------------|------------------|-------|---------------|
| 500 mg. of compound 1                                                                                                       | 1.59             | 0.04             | 1.34  | 100           |
| 500 mg. of compound 1 plus 100 mg. of H <sub>2</sub> N-CH <sub>2</sub> CH <sub>2</sub> NHCH <sub>2</sub> CH <sub>2</sub> OH | 1.55             | 0.04             | 1.04  | 126           |
| 500 mg. of compound 1 plus 100 mg. of H <sub>2</sub> N-CH <sub>2</sub> -CH-CH <sub>2</sub> -NH <sub>2</sub>                 | 1.54             | 0.05             | 1.10  | 128           |
| OH                                                                                                                          |                  |                  |       |               |
| NH <sub>2</sub>                                                                                                             | 1.55             | 0.05             | 1.00  | 123           |
| 500 mg. of compound 1 plus 100 mg. of H <sub>2</sub> N-(CH <sub>2</sub> ) <sub>8</sub> -CH-COOH-2HCl                        | 1.55             | 0.05             | 1.00  | 123           |

photosensitive element according to the invention as described in Example 5 in an amount of 100 mg per kg of emulsion, the speed is still further increased.

This is proved by the following results.

| Material                                                                             | Fresh material   |                  |       | Material stored for 5 days at 49°C/15 % R.H. |                  |              |
|--------------------------------------------------------------------------------------|------------------|------------------|-------|----------------------------------------------|------------------|--------------|
|                                                                                      | D <sub>max</sub> | D <sub>min</sub> | Gamma | D <sub>max</sub>                             | D <sub>min</sub> | Speed ma (%) |
| comparison material comprising 500 mg of compound 1                                  | 1.34             | 0.03             | 1.09  | 100                                          | 1.31             | 0.03         |
| material comprising 500 mg of compound 1 and 100 mg of the 3-pyrazolidinone compound | 1.35             | 0.03             | 1.17  | 129                                          | 1.42             | 0.03         |
|                                                                                      |                  |                  |       | 1.14                                         | 75               |              |

## EXAMPLE 7

Example 6 is repeated with the difference that now 45 per kg of emulsion 2 g of 1-phenyl-4,4-dimethyl-5-ethoxy-3-pyrazolidinone is used instead of 100 mg of 1-p-tolyl-4,4-dimethyl-5-ethoxy-3-pyrazolidinone.

The following results were attained with fresh material.

| Material                                                                          | D <sub>max</sub> | D <sub>min</sub> | Gamma | Speed(%) |
|-----------------------------------------------------------------------------------|------------------|------------------|-------|----------|
| Comparison material comprising 500 mg of compound 1                               | 1.52             | 0.04             | 1.35  | 100      |
| material comprising 500 mg of compound 1 and 2 g of the 3-pyrazolidinone compound | 1.67             | 0.03             | 1.90  | 142      |

These results also prove that the speed can still be further increased by 40 percent by adding to the emulsion in addition to the (poly)amino(poly)carboxylic acid a compound as described and claimed in United Kingdom Patent application 52,572/69, the maximum density of the image formed also being increased (by

25 We claim:

which comprises the steps of image-wise exposing a photosensitive element containing a silver halide emulsion layer, developing the exposed silver halide and forming a soluble silver complex of unexposed silver halide by treating the said silver halide emulsion layer 30 with an alkaline processing liquid in the presence of a hydroxylamine developing agent and a silver halide complexing agent, transferring said soluble silver complex by diffusion to an image-receiving element in superposed relationship with said photosensitive element, 35 forming at an image-receiving layer of said image-receiving element an image incorporating silver from said silver complex, and separating said image-receiving element from said photosensitive element, the use of a photosensitive element which includes in the silver halide emulsion layer or a hydrophilic colloid layer in water-permeable relationship with the said emulsion layer a (poly)amino(poly)carboxylic acid compound in the acid form or in the form of a water-soluble salt.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 826

15

present in the silver halide emulsion layer of the photosensitive element in an amount of from about 30 mg to 15 g per mole of silver halide.

6. A process according to claim 1, wherein said photosensitive element also includes an 1-aryl-3-pyrazolidinone compound.

7. A process according to claim 1, wherein said photosensitive element also includes a diamine or polyamine compound.

8. The process according to claim 1 wherein said (poly)amino(poly)carboxylic acid compound is ethylenediamine,N,N,N',N'-tetraacetic acid disodium salt.

9. The process according to claim 1 wherein said (poly)amino(poly)carboxylic acid compound is 15

16

ethylenediamine, N, N' - di(O - hydroxyamino (poly) carboxylic acid compound is ethylenediamine, N, N-di(O-hydroxyphenyl acetic acid.

10. The process according to claim 1 wherein said (poly)amino(poly)carboxylic acid compound is 2-hydroxyethyl-amino diacetic acid.

11. The process according to claim 1 wherein said (poly)amino(poly)carboxylic acid compound is ethyleneglycol bis(2-aminoethyl)-N,N,N',N'-tetraacetic acid.

12. The process according to claim 1 wherein said (poly)amino(poly)carboxylic acid compound is 2-hydroxy-3,5-dichlorobenzylamino-N-acetic acid sodium salt.

\* \* \* \* \*

20

25

30

35

40

45

50

55

60

65